

# UNITED STATES PATENT OFFICE.

HENRI SCHMID, OF MÜLHAUSEN, GERMANY, ASSIGNOR TO BADISCHE ANILIN & SODA FABRIK, OF LUDWIGSHAFEN-ON-THE-RHINE, GERMANY, A CORPORATION.

## PRODUCTION OF BROWN SHADES ON THE FIBER.

1,011,085.

Specification of Letters Patent.

Patented Dec. 5, 1911.

No Drawing.

Application filed November 30, 1909. Serial No. 530,658.

To all whom it may concern:

Be it known that I, HENRI SCHMID, chemist, citizen of the Swiss Republic, residing at Mülhausen, in Alsace, Germany, have invented new and useful Improvements in the Production of Brown Shades on the Fiber, of which the following is a specification.

In the specification of Letters Patent No. 863,761 is described the production of brown shades by oxidizing, on fibrous material by means of a chlorate in the presence of a vanadium salt, para-phenylene-diamin, or a homologue, or isomer, thereof, without sufficient mineral acid to combine with the whole thereof. This process, however, has the disadvantage that the shade of brown obtained cannot be sufficiently varied. I have now discovered that various shades of brown can be obtained if, when carrying out the aforesaid process, instead of para-phenylene-diamin alone, a mixture thereof with an amino-hydroxy compound be employed. When carrying out the process of this invention, both the para-phenylene-diamin body and the amino-hydroxy compound should be employed so that the whole thereof, or at any rate the greater part thereof, is in the form of the free base. When using such mixture of a para-phenylene-diamin body and an amino-hydroxy compound, results are obtained which cannot be obtained by the use of either of these constituents separately. For instance, although meta-amino-phenol when oxidized by itself on the material yields a light brown-violet shade, if it be oxidized in the presence of a limited quantity of para-phenylene-diamin, the shade produced is dark olive-brown. If a mixture of para-phenylene-diamin, ortho-amino-phenol, and meta-amino-phenol be employed, the brown compound produced has a yellowish tinge, whereas a mixture of para-phenylene-diamin and ortho-amino-phenol gives rise to a garnet shade of brown. Similarly, by taking other mixtures of para-phenylene-diamin, or a homologue, or isomer, thereof, with an amino-hydroxy-compound, other shades of brown can be obtained which are all fast against the action of washing and light. In each case variegated, or discharge, effects can be produced if desired.

The following are examples of the preparation of baths in accordance with my in-

vention, but the said invention is not limited to these examples.

*Example 1—Padding bath for brown.*—Dissolve ten grams of para-phenylene-diamin, four grams of ortho-amino-phenol, two grams of meta-amino-phenol, sixteen grams of ammonium chlorid, and sixteen grams of sodium chlorate, in water, add fifteen cubic centimeters of one per thousand ammonium vanadate solution, and make up the whole to one liter. If necessary, filter the solution. The bath can be used either before, or after, dilution.

*Example 2—Padding bath for fawn color.*—Dissolve nine grams of para-phenylene-diamin, five grams of meta-amino-phenol, one gram of ortho-amino-phenol, twenty grams of ammonium chlorid, and twenty grams of sodium chlorate in water, and add sixteen cubic centimeters of a one per thousand ammonium vanadate solution. Make up the whole to one liter and filter the solution, if necessary.

*Example 3—Padding bath for olive-brown.*—Dissolve seven grams of para-phenylene-diamin, seven grams of meta-amino-phenol, twenty grams of ammonium chlorid, and twenty grams of sodium chlorate in water, add sixteen grams of ammonium vanadate solution, and make up the whole to one liter.

The material, after being padded, or otherwise treated, with either of the aforesaid baths, should be dried rapidly, without being heated too strongly, and can then be steamed in a Mather-Platt apparatus, for example, if a uniform shade be desired.

Either white, or colored, discharge effects can be obtained, for example, in a manner similar to that described in the aforesaid specification of Letters Patent No. 863,761.

It is sometimes useful to add say from thirty to forty cubic centimeters of glycerin-tartar-emetic solution to each liter of the printing or padding solution. The glycerin-tartar-emetic solution can be prepared by dissolving forty grams of tartar emetic in six hundred and twenty cubic centimeters of hot water and three hundred and forty grams of glycerin.

Now what I claim is:

1. The process of producing brown shades on the fiber by applying to the material a mixture containing a para-phenylene-diamin

body and an amino-hydroxy body, a chlorate and a vanadium compound, at least one-half of the amino groups being in the free state, and then causing the oxidation of the para-phenylene-diamin body and of the amino-hydroxy body substantially as described.

2. The process of producing brown shades on the fiber by applying to the material a mixture containing para-phenylene-diamin and an amino-phenol and a chlorate and a vanadium compound, at least one-half of the amino groups being in the free state, and then causing the oxidation of the para-phenylene-diamin and of the amino-phenol substantially as described.

3. The process of producing brown shades on the fiber by applying to the material a mixture containing a para-phenylene-diamin body and an amino-hydroxy body, a chlorate and a vanadium compound, at least one-half of the amino groups being in the free state, then drying the material and subjecting it to the action of steam.

4. The process of producing brown shades with discharge effects on the fiber by applying to the material a mixture containing a para-phenylene-diamin body and an amino-hydroxy body, a chlorate and a vanadium compound, at least one-half of the amino groups being in the free state, then drying the material and printing with a paste con-

taining a reducing agent and then subjecting it to the action of steam.

5. The process of producing brown shades with discharge effects on the fiber by applying to the material a mixture containing a para-phenylene-diamin body and an amino-hydroxy body, a glycerin-tartar emetic solution, a chlorate and a vanadium compound, at least one-half of the amino groups being in the free state, then drying the material, printing it with a paste containing a reducing agent and then subjecting it to the action of steam.

6. The process of producing brown shades with discharge effects on the fiber by applying to the material a mixture containing a para-phenylene-diamin body and an amino-hydroxy body, a glycerin-tartar emetic solution, a chlorate and a vanadium compound, at least one-half of the amino groups being in the free state, then drying the material, printing it with a paste containing a reducing agent and a coloring matter, and then subjecting it to the action of steam.

In testimony whereof I have hereunto set my hand in the presence of two subscribing witnesses,

HENRI SCHMID.

Witnesses:

GEORGE GIFFORD,  
ARNOLD ZÜBER.